# EUROPEAN PATENT SPECIFICATION

(11) **EP 2 156 898 B1**
(45) Date of publication and mention of the grant of the patent: **31.07.2013**
(21) Application number: 09014312.4
(22) Date of filing: 08.09.2005
(51) Int. Cl.: B05C 5/00, B05D 1/30

(54) **Curtain coating system**
Vorhangbeschichtungsvorrichtung
Dispositif de revêtement de rideau

(30) Priority: 09.09.2004 US 608213 P
(43) Date of publication of application: 24.02.2010
(62) Divisional of application: 05791609.0
(73) Proprietor: Avery Dennison Corporation, Pasadena, CA 91103-3596 (US)
(72) Inventor: Jansen, Alexander, Pasadena, CA 91103 (US); Fermin, Robert J., Pasadena, CA 91103 (US); Wang, Chunhwa E., Pasadena, CA 91103 (US)
(74) Representative: Müller-Boré & Partner Patentanwälte

(56) References cited:
- EP-A- 0 197 493
- EP-A- 0 969 147
- WO-A-92/11571
- WO-A1-03/049870
- DE-A1- 10 012 344
- DE-A1- 10 057 731
- DE-A1- 19 735 980
- JP-A- 8 084 951
- JP-A- 8 201 961

## Description

### FIELD OF THE INVENTION

The present invention relates generally, as indicated, to a curtain coating system and, more particularly, to a system wherein a moving substrate is impinged by a free-falling curtain of a liquid coating composition as the substrate passes through an impingement zone.

### DEFINITIONS

The coating weight (ctwt) is the weight of the dried coating on the substrate and is expressed in dimensions of mass per area. (*e.g.,* kg/m²).

The density (ρ) is the density of the liquid coating composition and is expressed in dimensions of mass per volume (*e.g.,* kg/m³).

The predetermined uniform coating thickness (t_{∞}) is the thickness (or height) of the liquid coating composition if perfectly applied and is expressed in dimensions of length (*e.g.,* mm).

The final coating thickness (t_{w}) is the actual thickness of the liquid coating on any particular point across the width of the coating and is expressed in dimensions of length (*e.g.,* mm).

The substrate velocity (U) is the velocity of the substrate through the impingement zone and is expressed in dimensions of length per time (*e.g.,* m/min).

The downstream direction (D) is the direction of the substrate as it passes through the impingement zone and is dimensionless.

The impingement velocity (V) is the velocity of the curtain just prior to contacting the substrate in the impingement zone and is expressed in dimensions of length per time (*e.g.,* m/s).

The gravitational acceleration (g) is a constant representing the acceleration caused by gravity and is expressed in length per time-squared (*e.g.,* 9.81 m/s²).

The initial velocity (V₀) is the initial velocity of the curtain at die-lip-detachment and is expressed in dimensions of length per time (*e.g.,* m/s).

The impingement angle (θ) is the angle between a vector representing gravity (*i.e*., a vertical vector) and a downstream portion of a vector tangential to, or parallel with, the substrate as it passes through the impingement zone and is expressed dimensions of angular units (*e.g.,* degrees).

The horizontal component Uₓ, is the horizontal component of the substrate velocity (U) (*i.e*., Uₓ = Usinθ) and is expressed in dimensions of length per time (*e.g*., m/min).

The vertical component Uy is the vertical component of the substrate velocity (U) (*i.e.,* U_{y} = Ucosθ) and is expressed in dimensions of length per time (*e.g.,* m/min.)

The parallel impingement component (V_{∥}) is the component of the impingement velocity (V) positioned parallel with the substrate velocity (U) (*i.e.,* V_{∥} = Vsinθ) and is expressed in dimensions of length per time (*e.g.,* m/s).

The perpendicular impingement component (V_{⊥}) is the component of the impingement velocity (V) positioned perpendicular with the substrate velocity (U), (*i.e.,* V_{⊥} = Vsinθ) and is expressed in dimensions of length per time (*e.g.,* m/s).

The speed ratio (SP) is the ratio of the substrate velocity (U) to the perpendicular impingement component (V_{⊥}) and is dimensionless.

The width (w) is the lateral cross-wise dimension of the curtain and is expressed in dimensions of length (*e.g.,* m).

The height (h) is the vertical dimension of the curtain from die-lip-detachment to the impingement zone and is expressed in dimensions of length (*e.g.,* cm).

The volumetric flow rate per unit width (Q) is the volumetric flow rate of the curtain divided by the width (w) of the curtain and is expressed in dimensions of volume per time and length (*e.g.,* kg/s*m).

The mass flow rate per unit width (p*Q) is the product of the volumetric flow rate (Q) and the density (ρ) of the liquid coating composition forming the curtain and is expressed in dimensions of mass per unit time and length (*e.g.,* kg/s*m).

The viscosity (η) is the viscosity of the liquid coating composition within the impingement zone at a shear rate of 10,000 1/s and is expressed in dimensions of mass per length and time (*e.g.,* kg/m*s or Pa*s).

The force ratio or Reynolds' number (Re) is the ratio of the mass flow rate per unit width of the curtain (ρ*Q) to the viscosity (n) of the liquid coating composition and is dimensionless.

### BACKGROUND OF THE INVENTION

A curtain coating method generally comprises impinging a moving substrate with a free-falling curtain of a liquid coating composition as the substrate passes through an impingement zone. A customer will typically specify a certain substrate (*e.g.,* paper or plastic film), a particular coating composition (*e.g.,* adhesive coating) and a desired coating weight (ctwt). The selected coating composition will have a density (ρ), a percent solids (%), and a viscosity (η). For example, an adhesive coating composition will have a density (ρ) between about 900 kg/m³ and about 1100 kg/m³ and a viscosity (η) between about 0.040 Pa*s and about 0.160 Pa*s. If the liquid coating composition were perfectly applied, the coating would have a predetermined uniform thickness (t_{∞}) equal to the coating weight (ctwt) divided by the percent of solids (%) and the density (ρ) of the liquid coating composition.

The substrate moves through the impingement zone at a certain substrate velocity (U) and the curtain contacts the substrate at an impingement velocity (V). A conveyor controls the substrate speed and generally allows this speed to be set between at least about 300 m/min and about 1000 m/min. The impingement velocity (V) controlled by gravitational acceleration (g) and can be calculated from the curtain's initial velocity (V₀) at die-lip-detachment and its height (h) from die-lip-detachment to the impingement zone. (*i.e*., V = V₀ + (2gh)^{½}). Thus, for example, if a curtain has a height (h) of about 15 cm and an initial velocity (V₀) of about zero, the impingement velocity will be about 1.72 m/s.

The curtain has a certain volumetric flow rate per unit width (Q) at the impingement zone. The volumetric flow rate (Q) should equal the product of the substrate velocity (U) and the predetermined uniform coating thickness (t_{∞}). As was noted above, a customer will specify a particular coating composition (and thus a particular density (ρ) and a particular percent solids (%)) and a desired coating weight (ctwt), and thus essentially specifies a predetermined uniform coating thickness (t_{∞}). Accordingly, for a given coating composition and a given coating weight (ctwt), a reduction in the volumetric flow rate (Q) results in a corresponding reduction of substrate velocity (U).

A curtain's flow characteristics at the impingement zone can be expressed in terms of the ratio of its inertia force (ρ*Q) to its viscous force (η), that is its Reynolds number (Re). Thus, for a particular customer-specified coating composition, the force ratio (Re) can be raised and lowered by increasing and decreasing, respectively, the volumetric flow rate (Q).

A curtain coating method can only be successfully performed upon the correct correlation of curtain coating parameters, including substrate velocity (U), impingement velocity (V), and force ratio (Re). If a curtain coating method is successfully performed, the substrate will be provided with an extremely consistent and precise coating over thousands of meters of substrate length. Specifically, for example, the coating will have a thickness (t_{w}) that varies very little (*e.g.,* less than 2%, less than 1.5%, less than 1.0% and/or less than 0.5%) from the predetermined uniform coating thickness (t_{∞}) over the width (w) of the coating.

In the past, curtain coating has not been successful at relatively high force ratios (*e.g.,* greater than 5.25). This problem has been solved or, perhaps more accurately, avoided, by decreasing the volumetric flow rate (Q) to thereby red uce the force ratio (Re). As was noted above, for a given customer-specified coating weight (ctwt), a relatively low volumetric flow rate (Q) requires a relatively low substrate velocity (U).

The substrate velocity (U) is the overall production speed for the curtain coating process. The higher the substrate velocity (U), the more efficient the manufacturing process. Accordingly, from an economic point of view, a high substrate velocity (U) is preferred as it best maximizes the productivity of capital-investment curtain coating equipment. However, the inability to successfully curtain coat at high force ratios (Re) has resulted in the industry settling for relatively low volumetric flow rates (Q) and thus relatively low substrate velocities (U).

WO 92/11571 discloses a method for coating a support, such as a web or film, with a liquid composition, such as a photographic emulsion. The support is moved through a coating zone and a moving sheet of the composition is directed at the support.

### SUMMARY OF THE INVENTION

According to the present invention, a curtain coating system having the features disclosed in claim 1 is provided. Preferred embodiments are defined in the dependent claims.

### DRAWINGS

Figures 1A and 1B are schematic views of curtain coating methods wherein the impingement angle (θ) is approximately equal to 90°.
Figure 2 is a close-up schematic view of a successfully curtain-coated product.
Figures 3A and 3B are schematic views of the substrate velocity (U) vector and the impingement velocity (V) vector at the impingement zone in the curtain coating methods shown in Figures 1A and 1B, respectively.
Figure 4A and 4B are schematic views of curtain coating methods wherein the impingement angle (θ) is less than 90°.
Figures 5A and 5B are schematic views of the substrate velocity (U) vector and the impingement velocity (V) vector at the impingement zone in the curtain coating methods shown in Figures 5A and 5B, respectively.
Figures 6A and 6B are front schematic views of edge guides for the curtain coating systems shown in Figures 1A-1B and Figure 4A-4B, respectively.
Figure 7 is a schematic view of a vacuum assembly modified to accommodate the curtain coating system shown in Figure 4A.
Figures 8A and 8B are side schematic views of die lips for the curtain coating systems shown in Figures 1A-1B and Figure 4A-4B, respectively.

### TABLES

Table 1 is a compilation of raw data collected during curtain coating runs at various substrate velocities (U) and impingement angles (θ), the data being sorted by run number.
Table 2A is a compilation of the speed ratios (SP) and the force ratios (Re) during curtain coating runs when the impingement angle (θ) was equal to 90°, the data being sorted by speed ratios (SP).
Table 2B is a compilation of the speed ratios (SP) and the force ratios (Re) during curtain coating runs when the impingement angle (θ) was equal to 90°, the data being sorted by force ratios (Re).
Table 3A is a compilation of the speed ratios (SP) and the force ratios (Re) during curtain coating runs when the impingement angle (θ) was equal to 65°, the data being sorted by speed ratios (SP).
Table 3B is a compilation of the speed ratios (SP) and the force ratios (Re) during curtain coating runs when the impingement angle (θ) was equal to 65°, the data being sorted by force ratios (Re).
Table 4A is a compilation of the speed ratios (SP) and the force ratios (Re) during curtain coating runs when the impingement angle (θ) was equal to 60°, the data being sorted by speed ratios (SP).
Table 4B is a compilation of the speed ratios (SP) and the force ratios (Re) during curtain coating runs when the impingement angle (θ) was equal to 60°, the data being sorted by force ratios (Re).
Table 5A is a compilation of the speed ratios (SP) and the force ratios (Re) during curtain coating runs when the impingement angle (θ) was equal to 55°, the data being sorted by speed ratios (SP).
Table 5B is a compilation of the speed ratios (SP) and the force ratios (Re) during curtain coating runs when the impingement angle (θ) was equal to 55°, the data being sorted by force ratios (Re).
Table 6A is a compilation of the speed ratios (SP) and the force ratios (Re) during curtain coating runs when the impingement angle (θ) was equal to 90°, 65°, 60°, and 55°, the data being sorted by speed ratios (SP).
Table 6B is a compilation of the speed ratios (SP) and the force ratios (Re) during curtain coating runs when the impingement angle (θ) was equal to 90°, 65°, 60°, and 55°, the data being sorted by force ratios (Re).

### GRAPHS

Graph 1 A is a plot of the relationship between the speed ratio (SP) and the force ratio (Re) when the impingement angle (θ) is equal to 90°.
Graph 1B is a plot of the relationship between the substrate velocity (U) and the force ratio (Re) when the impingement angle (θ) is equal to 90°.
Graph 2A is a plot of the relationship between the speed ratio (SP) and the force ratio (Re) when the impingement angle (θ) is equal to 65°.
Graph 2B is a plot of the relationship between the substrate velocity (U) and force ratio (Re) when the impingement angle (θ) is equal to 65°.
Graph 3A is a plot of the relationship between the speed ratio (SP) and the force ratio (Re) when the impingement angle (θ) is equal to 60°.
Graph 3B is a plot of the relationship between the substrate velocity (U) and the force ratio (Re) when the impingement angle (θ) is equal to 60°.
Graph 4A is a plot of the relationship between the speed ratio (SP) and the force ratio (Re) when the impingement angle (θ) is equal to 55°.
Graph 4B is a plot of the relationship between the substrate velocity (U) and the force ratio (Re) when the impingement angle (θ) is equal to 55°.

### DETAILED DESCRIPTION

Referring now to the drawings, and initially to Figures 1A and 1B, a system 10 for performing a curtain coating method is schematically shown. The method generally comprises the steps of conveying a substrate 12 in a downstream direction (D) through an impingement zone 14, and impinging the substrate 12 with a free-falling curtain 16 in the impingement zone 14 at an impingement angle (θ) to form a coating 18 on the substrate 12 of a desired coating weight (ctwt). As is best seen by referring briefly to Figure 2, if the curtain coating method is successfully performed, the substrate 12 will be provided with a coating 18 having a thickness (t_{w}) that varies less than 2%, that varies less than 1.5%, that varies less than 1.0%, and/or that varies less than 0.5% from the predetermined uniform coating thickness (t_{∞}) over the width (w) of the coating 18.

The substrate 12 moves through the impingement zone 14 at a substrate velocity (U) and the curtain 16 contacts the substrate 12 at a impingement velocity (V). A conveyor controls the substrate velocity (U) and allows the speed (U) to be set between at least about 300 m/min and about 1000 m/min. In Figure 1A, the conveyor comprises a back-up roll 22 around which the substrate 12 is moved, and, in Figure 1B, the conveyor comprises two horizontally spaced rolls 24 between which the substrate12 is moved. The curtain 16 can be formed by the liquid coating composition falling from a die 20 and the curtain 16 contacts the substrate 12 at an impingement velocity (V). If, for example, the curtain 16 has a height (h) of about 15 cm and its initial velocity (V₀) is about zero, the impingement velocity (V) will be about 1.72 m/s.

As is best seen by referring additionally to Figures 3A and 3B, (schematically showing the substrate velocity (U) vector and the impingement velocity (V) vector), the curtain 16 contacts the impingement zone 14 at an impingement angle (θ). In Figure 3A (corresponding to Figure 1A), the impingement angle (θ) is the angle between a first line representing gravity (*i.e.,* a vertical line) and a second line tangent to the top-dead-center of the back-up roll 22. In Figure 3B (corresponding to Figure 1 B), the impingement angle (θ) is the angle between a first line representing gravity (*i.e.,* a vertical line) and a second line parallel to the path created by the conveying rollers 24. In both cases, the second line is horizontal and thus the impingement angle (θ) is equal to 90°.

In the curtain coating system shown in Figures 1A and 1B, speed ratios (SP) between about 3 and about 10 can provide successful curtain coating. Specifically, speed ratios (SP) between about 3 and about 4 (*e.g.,* a range contained within the area defined by data points having x-coordinates 2.91, 3.88, 4.85) can accommodate force ratios (Re) from about 1.0 to about 3.5. For an impingement velocity (V) of about 1.72 m/s, this corresponds to a substrate velocity (U) between about 300 m/min and about 500 m/min. For an adhesive coating composition (having a density (ρ) between about 900 kg/m³ and about 1100 kg/m³ and having a viscosity (η) between about 0.040 Pa*s and about 0.160 Pa*s) this corresponds to a volumetric flow rate range (Q) of about 0.00004 m³/(s*m) to about 0.0006 m³/(s*m). (See Tables 2A-2B and 6A-6B, see Graphs 1A-1B.)

Speed ratios (SP) between about 4 and about 5 (*e.g.,* a range contained within the area defined by data points having x-coordinates 3.88, 4.85, 5.81) can accommodate force ratios (Re) from about 1.8 up to about 4.2. For an impingement velocity (V) equal to about 1.72 m/s, this corresponds to a substrate velocity (U) between about 400 m/min and about 600 m/min. For an adhesive coating composition, this corresponds to a volumetric flow rate (Q) range of about 0.000065 m³/(s*m) to about 0.00075 m³/(s*m). (See Tables 2A-2B, 6A-6B, and see Graphs 1A-1B.)

Speed ratios (SP) between about 5 and 6 (*e.g.,* a range contained within the area defined by data points having x-coordinates 4.85, 5.81 and 6.78) can accommodate force ratios (Re) from about 1.9 up to about 5.0. For an impingement velocity (V) equal to about 1.72 m/s, this corresponds to a substrate velocity (U) between about 500 m/min and about 700 m/min. For an adhesive coating composition, this corresponds to a volumetric flow rate (Q) range of about 0.00007 m³/(s*m) to about 0.00089 m³/(s*m). (See Tables 2A-2B, 6A-6B and see Graphs 1A-1 B.)

Speed ratios (SP) between about 6 and 7 (*e.g.,* a.range contained within the area defined by data points having x-coordinates 5.81, 6.78, 7.75) can accommodate force ratios (Re) from about 2.1 up to about 5.2. For an impingement velocity (V) equal to about 1.72 m/s, this corresponds to a substrate velocity (U) between about 600 m/min and about 800 m/min. For an adhesive coating composition, this corresponds to a volumetric flow rate (Q) range of about 0.000076 m³/(s*m) to about 0.00092 m³/(s*m). (See Tables 2A-2B, 6A-6B, and see Graphs 1A-1B.)

Speed ratios (SP) between 7 and 8 (*e.g.,* a range contained within the area defined by data points having x-coordinates 6.78, 7.75, 8.72) can accommodate force ratios (Re) from about 2.3 to about 5.2. For an impingement velocity (V) equal to about 1.72 m/s, this corresponds to a substrate velocity (U) between about 700 m/min and about 900 m/min. For an adhesive coating composition , this corresponds to a volumetric flow rate (Q) range of about 0.00008 m³/(s*m) to about 0.00092 m³/(s*m). (See Tables 2A-2B, 6A-6B, and see Graphs 1A-1B.)

Speed ratios (SP) between 8 and 9 (*e.g.,* a range contained within the area defined by data points having x-coordinates 7.75, 8.72, 9.69) can accommodate force ratios (Re) from about 2.7 to about 5.2. For an impingement velocity (V) equal to about 1.72 m/s, this corresponds to a substrate velocity (U) between about 800 m/min and about 900 m/min. For an adhesive coating composition, this corresponds to a volumetric flow rate (Q) range of about 0.000098 m³/(s*m) to about 0.00092 m³/(s*m). (See Tables 2A-2B, 6A-6B and see Graphs 1A-1B.)

Speed ratios (SP) between 9 and 10 (*e.g.,* a range contained within the area defined by data points having x-coordinates 8.72 and 9.69) can accommodate force ratios (Re) from about 3.0 to about 5.2. For an impingement velocity (V) equal to about 1.72 m/s, this corresponds to a substrate velocity (U) between about 900 m/min and about 1000 m/min. For an adhesive coating composition, this corresponds to a volumetric flow rate (Q) range of about 0.000109 m³/(s*m) to about 0.00092 m³/(s*m). (See Tables 2A-2B, 6A-6B and see Graphs 1A-1 B.)

Thus, speed ratios (SP) between about 3 and about 10 can provide successful curtain coating when the impingement angle (θ) is equal to about 90°. However, speed ratios (SP) between about 3 and about 10 cannot provide successful coating at higher force ratios (Re), that is force ratios (Re) greater than 5.25. (See Tables 2A-2B, 6A-6B, and see Graphs 1A-1 B.)

Curtain coating was unsuccessful at high force ratios (Re) because a substantial bank of liquid (*i.e.,* a heel) forms upstream of the impingement zone 14 and, in some cases, air is trapped thereunderneath. Heel formation results in undulated and uneven coating thickness, and excessive air entrapment results in coating-void regions (*e.g.,* empty spots/stripes on the substrate). This leads to an unacceptable level of cross-web defects and the coating 18 having a thickness (t_{w}) that varies 2% or more from the desired final uniform coating thickness (t_{∞}) over the width (w) of the coating 18.

In the past, this problem has been avoided by decreasing the volumetric flow rate (Q) (to thereby reduce the force ratio (Re)) and thus reducing the substrate velocity (U) and compromising the efficiency of the curtain coating process. For example, with an adhesive coating composition, the volumetric flow rate (Q) is limited to 0.00092 m³/(s*m) even if the coating composition has a relatively low density (ρ) (*e.g.,* 900 kg/m³) and a relatively high viscosity (*e.g.,* 0.160 Pa*s).

With a low viscosity coating composition, such as release coating (*e.g*. a coating composition having a density (ρ) between about 900 kg/m³ and about 1100 kg/m³ and having a viscosity (η) between about 0.005 Pa*s and about 0.015 Pa*s), the volumetric flow rate (Q) is believed to be even more limited. Specifically, for example, speed ratios (SP) between about 3 and about 4 and force ratios (Re) from about 1.0 to about 3.5 would correspond to a volumetric flow rate (Q) range of about 0.000005 m³/(s*m) to about 0.00006 m³/(s*m). Speed ratios (SP) between about 4 and about 5 and force ratios (Re) from about 1.8 up to about 4.2 would correspond to a volumetric flow rate (Q) range of about 0.000008 m³/(s*m) to about 0.00007 m³/(s*m). Speed ratios (SP) between about 5 and 6 and force ratios (Re) from about 1.9 up to about 5.0 would correspond a volumetric flow rate (Q) range of about 0.000009 m³/(s*m) to about 0.00008 m³/(s*m). Speed ratios (SP) between about 6 and 7 and force ratios (Re) from about 2.1 up to about 5.2 would correspond to a volumetric flow rate (Q) range of about 0.000010 m³/(s*m) to about 0.000087 m³/(s*m). Speed ratios (SP) between 7 and 8 and force ratios (Re) from about 2.3 to about 5.2 would correspond to a volumetric flow rate (Q) range of about 0.000010 m³/(s*m) to about 0.000087 m³/(s*m). Speed ratios (SP) between 8 and 9 and force ratios (Re) from about 2.7 to about 5.2 would correspond to a volumetric flow rate (Q) range of about 0.000012 m³/(s*m) to about 0.000087 m³/(s*m). Speed ratios (SP) between 9 and 10 and force ratios (Re) from about 3.0 to about 5.2 would correspond to a volumetric flow rate (Q) range of about 0.000014 m³/(s*m) to about 0.000087 m³/(s*m). Thus, with a release coating composition, the volumetric flow rate (Q) can be limited to 0.000087 m³/(s*m) even if the coating composition has a relatively low density (ρ) (*e.g.,* 900 kg/m³) and a relatively high viscosity (*e.g.,* 0.015 Pa*s).

Referring now to Figures 4A and 4B, a curtain coating system according to the present invention is schematically shown. This curtain coating system 10 is the same as that discussed above (whereby like references are used) except that the impingement angle (θ) is not equal to 90°. Instead, the impingement angle (θ) is less than 90°, not greater than about 65°, not greater than about 60°, not greater than about 55°, is between about 70° and about 50° and/or is between about 65° and about 55°. In Figure 4A, the impingement zone 14 is offset in the downstream direction (D) from the top-dead-center of the back-up roller 22. In Figure 4B, the conveying rollers 24 are vertically offset to slope in the downstream direction (D).

As is best seen by referring additionally to Figures 5A and 5B, the impingement velocity (V) vector can be viewed as having a component (V_{⊥}) perpendicular to the substrate velocity (U) vector and a component (V_{∥}) parallel to the substrate velocity (U) vector. The perpendicular component (V_{⊥}) corresponds to the sine of the impingement angle (V_{⊥} = Vsinθ) and the parallel component (V_{∥}) corresponds to the cosine of the impingement angle (V_{∥} = Vcosθ). Also, the substrate velocity (U) vector can be viewed as having a horizontal component (Uₓ), corresponding to the sine of the impingement angle (Uₓ = Usinθ), and a vertical component (U_{y}), corresponding to the cosine of the impingement angle (U_{y} = Ucosθ).

The present invention includes the appreciation that the most telling speed ratio (SP) is not simply be the ratio (UN) of the substrate velocity (U) to the impingement velocity (V), but rather a ratio properly representing the velocity shift at the impingement zone 14. Specifically, the parallel component (V_{∥}) of the impingement velocity (V) does not necessitate any velocity shift at the impingement zone 14. Likewise, only the perpendicular component (V_{⊥}) of the impingement velocity (V) vector requires a velocity shift in the impingement zone 14. Accordingly, the important dimensionless speed ratio (SP) is the ratio of the substrate velocity (U) to the perpendicular component (V_{⊥}) of the impingement velocity (V). It may be noted that when the impingement angle (θ) was equal to 90° (Figures 1A/3A and 1B/3B, and Tables 2A-2B), the perpendicular component (V_{⊥}) was equal to the impingement velocity (V) and the speed ratio (SP) reduced to the ratio of the substrate speed (U) to the impingement speed (V).

The present invention also includes the appreciation that the vertical component (U_{y}) of the substrate velocity (U) is significant in that it provides a gravitational "push" or downward momentum to the impinging liquid coating composition. While not wishing to be bound by theory, this "push" is believed to move otherwise heel-forming and/or air-entrapping impinging liquid through the impingement zone. It may be noted that when the impingement angle (θ) was equal to 90°, the vertical component (U_{y}) of the substrate velocity (U) was equal to zero and such a "push" was not provided to the impinging liquid.

Successful curtain coating can be accomplished at higher force ratios (Re) when the impingement angle (θ) is less than 90°, and in the tabulated/graphed embodiment of the invention, is equal to about 65°, about 60°, and/or about 55°. Specifically, for example, curtain coating was successful even when the curtain Reynold's number (Re) exceeded about 5.25, exceeded about 5.50, exceeded 6.00, exceeded 6.50, exceeded 7.00, exceeded 7.50, and/or exceeded 8.00. (See Tables 3A, 4A, 5A, 6A and see Graphs 2A, 3A, 4A.)

Specifically, force ratios (Re) from about 5.2 to about 6.0 (*e.g.,* a range contained within the area defined by the data points having y-coordinates 5.220, 5.510, 5.766, 5.966, 6.198) are compatible with speed ratios (SP) between about 7.5 and about 9.5. For an impingement velocity (V) of about 1.72 m/s, this corresponds to a substrate velocity (U) range of about 700 m/min to about 800 m/min. For an adhesive coating composition (*e.g*. a coating composition having a density (ρ) between about 900 kg/m³ and about 1100 kg/m³ and having a viscosity (n) between about 0.040 Pa*s and about 0.160 Pa*s) this corresponds to a volumetric flow rate (Q) range of about 0.000189 m³/(s*m) to about 0.00107 m³/(s*m). (See Tables 3A-3B, 4A-4B, 5A-5B, 6A-6B and see Graphs 2A-2B, 3A-3B, 4A-4B.)

Force ratios (Re) between about 6 and 7 (*e.g.,* a range contained within the area defined by the data points having y-coordinates 5.966, 6.198, 6.590, 6.712, 6.887, 7.414) are compatible with speed ratios (SP) between about 8.6 and about 11.9. For an impingement velocity of about 1.72 m/s, this corresponds to an about 800 m/min to about 1000 m/min substrate velocity (U) range. For an adhesive coating composition, this corresponds to a volumetric flow rate (Q) range of about 0.000218 m³/(s*m) to about 0.00124 m³/(s*m). (See Tables 3A-3B, 4A-4B, 5A-5B, 6A-6B and see Graphs 2A-2B, 3A-3B.)

Force ratios (Re) between about 7 and 8 (*e.g.,* a range contained within the area defined by the data points having y-coordinates 6.887, 7.414, 7.458, 8.238) are compatible with speed ratios (SP) between about 9.6 and 11.9. For an impingement velocity (V) of about 1.72 m/s, this corresponds to an about 900 m/min to about 1000 m/min substrate velocity (U) range. For an adhesive coating composition, this corresponds to a volumetric flow rate (Q) range of about 0.000255 m³/(s*m) to about 0.00142 m³/(s*m). (See Tables 3A-3B, 4A-4B, 5A-5B, 6A-6B and see Graphs 2A-2B, 3A-3B, 4A-4B.)

Force ratios (Re) above 8 (*e.g.,* a range contained within the area defined by the data points having y-coordinates 8.238) are compatible with speed ratios (SP) between about 10.7 and about 11.9 For an impingement velocity (V) of about 1.72 m/s, this corresponds to an about 1000 m/min substrate velocity (U). For an adhesive coating composition, this corresponds to a volumetric flow rate (Q) as high as 0.0147 m³/(s*m) if the coating composition has a relatively low density (ρ) (*e.g.,* 900 kg/m³) and a relatively high viscosity (*e.g.,* 0.160 Pa*s). (See Tables 3A-3B, 4A-4B, 5A-5B, 6A-6B and see Graphs 2A-2B, 3A-3B, 4A-4B.).

With a low viscosity coating composition, such as a release coating (*e.g*. a coating composition having a density (ρ) between about 900 kg/m³ and about 1100 kg/m³ and having a viscosity (η) between about 0.005 Pa*s and about 0.015 Pa*s), similar flow rate (Q) increases are believed to be obtainable with the present invention. Specifically, force ratios (Re) from about 5.2 to about 6.0 and speed ratios (SP) between about 7.5 and about 9.5 correspond to a volumetric flow rate (Q) range of about 0.000024 m³/(s*m) to about 0.000100 m³/(s*m). Force ratios (Re) between about 6 and 7 and speed ratios (SP) between about 8.6 and about 11.9 correspond to a volumetric flow (Q) range of about 0.000027 m³/(s*m) to about 0.000117 m³/(s*m). Force ratios (Re) between about 7 and 8 and speed ratios (SP) between about 9.6 and 11.9 correspond to a volumetric flow (Q) range of about 0.000032 m³/(s*m) to about 0.000133 m³/(s*m). Force ratios (Re) above 8 and speed ratios (SP) between about 10.7 and about 11.9 correspond to volumetric flows from about 0.000036 m³/(s*m) to above 0.000136 m³/(s*m).

Speed ratios (SP) between about 7.5 and about 8.0 (*e.g.,* a range contained within the area defined by the data points having x-coordinates 7.48, 7.83, 8.28) can accommodate force ratios (Re) up to about 5.9 (*e.g.,* less than about 6.0). Speed ratios (SP) between about 8.0 and 9.0 (*e.g.,* a range contained within the area defined by the data points having x-coordinates 7.83, 8.28, 8.55, 8.95, 9.46) can accommodate force ratios (Re) up to about 6.8 (*e.g.,* less than about 7.0). Speed ratios (SP) between about 9.0 and 10.5 (*e.g.,* a range contained within the area defined by the data points having x-coordinates 8.95, 9.46, 9.62, 10.07, 10.65) can accommodate force ratios (Re) up to about 7.4 (*e.g.,* less than about 7.5). Speed ratios (SP) between about 10.5 and 12.0 (*e.g.,* a range contained within the area defined by the data points having x-coordinates 10.07, 10.65, 10.69, 11.19, 11.83) can accommodate force ratios (Re) up to about 8.2 (*e.g.,* less than 8.5). (See Tables 3B, 4B, 5B, 6B and see Graphs 2B, 3B, 4B.)

Substrate velocities (U) having horizontal components (Uₓ) between about 600 m/min and about 900 m/min can accommodate force ratios (Re) greater than 5.25. Specifically, horizontal components (Uₓ) between about 600 m/min and about 700 m/min (*e.g.,* a range contained within the area defined by the data points having x-coordinates 573, 606, 634, 655, 693, 725) can accommodate force ratios (Re) up to about 6.6 (*e.g.,* less than 7.0). Horizontal components (Uₓ) between about 700 m/min and about 800 m/min (*e.g.,* a range contained within the area defined by the data points having x-coordinates 693, 725, 737, 779, 816) can accommodate force ratios (Re) up to about 7.4 (*e.g.,* less than 7.5). Horizontal components (Uₓ) between about 800 m/min and about 900 m/min (*e.g.,* a range contained within the area defined by the data points having x-coordinates 779, 816, 866, 906) can accommodate force ratios (Re) up to about 8.2 (*e.g.,* less than 8.5).

Substrate velocities (U) having vertical components (U_{y}) between about 300 m/min and about 600 m/min can accommodate force ratios (Re) greater than 5.25. Specifically, vertical components (U_{y}) between about 300 m/min and about 350 m/min (*e.g.,* a range contained within the area defined by the data points having x-coordinates 296, 338, 350, 380) can accommodate force ratios (Re) up about 6.6 (*e.g.,* less than about 7.0). Vertical components (U_{y}) between about 350 m/min and about 400 m/min (*e.g.,* a range contained within the area defined by the data points having x-coordinates 338, 350, 380, 400, 402) can accommodate force ratios (Re) up about 7.4 (*e.g.,* less than about 7.5). Vertical components (U_{y}) between about 400 m/min and about 600 m/min (*e.g.,* a range contained within the area defined by the data points having x-coordinates 380, 400, 402, 423, 450, 459, 500, 516, 574) can accommodate force ratios (Re) up to at least about 8.2 (*e.g.,* less than about 8.5).

Impingement velocities (V) having perpendicular components (V_{⊥}) between about 1.4 m/s and about 1.6 m/s (*e.g.* a range contained within the area defined by the data points having x-coordinates 1.41,1.49,1.56) can accommodate force ratios (Re) greater than 5.25 and up to at least 8.2. Impingement velocities (V) having parallel components (V_{∥}) between about 0.7 m/s and about 1.0 m/s (*e.g*. a range contained within the area defined by the data points having x-coordinates 0.73,0.86, 0.99) can accommodate high ratios (Re) greater than 5.25 and up to at least 8.2. Successful curtain coating was obtained at these impingement velocity components (V_{⊥},V_{∥}) when the substrate velocity (U) was between about 700 m/min and 1000 m/min, when the horizontal component (Uₓ) of the substrate velocity (U) was between about 570 m/min and 910 m/min, and when the vertical component (U_{y}) of the substrate velocity (U) was between about 300 m/min and about 600 m/min.

Significantly, curtain coating was also successful at lower force ratios (Re) for these acute impingement angles. Specifically, force ratios (Re) between about 1 and 2 (*e.g.,* a range contained within the area defined by the data points having y-coordinates 1.01, 1.34, 1.68, and 2.02) are compatible with speed ratios (SP) between about 3.2 and about 6.4. For an impingement velocity (V) of about 1.72 m/s, this corresponds to an about 300 m/min to 600 m/min substrate velocity (U) range. For an adhesive coating composition (*e.g*. a coating composition having a density (ρ) between about 900 kg/m³ and about 1100 kg/m³ and having a viscosity (η) between about 0.040 Pa*s and about 0.160 Pa*s) this corresponds to a volumetric flow rate (Q) range of about 0.000036 m³/(s*m) to about 0.000356 m³/(s*m). For a release coating composition (*e.g*. a coating composition having a density (ρ) between about 900 kg/m³ and about 1100 kg/m³ and having a viscosity (η) between about 0.005 Pa*s and about 0.015 Pa*s) this corresponds to a volumetric flow rate (Q) range of about 0.000005 m³/(s*m) to about 0.000033 m³/(s*m). (See Tables 3A, 4A, 5A, 6A and see Graphs 2A, 3A, 4A.)

Force ratios (Re) between about 2 and 3 (*e.g.,* a range contained within the area defined by the data points having y-coordinates 1.68, 2.02, 2.06, 2.24, 2.35, 2.47, 2.69, 2.76, 2.98, 3.02) are compatible with speed ratios (SP) between about 3.2 and about 9.6. For an impingement velocity (V) of about 1.72 m/s, this corresponds to an about 300 m/min to about 900 m/min substrate velocity (U) range. For an adhesive coating composition, this corresponds to a volumetric flow rate (Q) range of about 0.000073 m³/(s*m) to about 0.000533 m³/(s*m). For a release coating composition, this corresponds to a volumetric flow rate (Q) range of about 0.000009 m³/(s*m) to about 0.000050 m³/(s*m). (See Tables 3A, 4A, 5A, 6A and see Graphs 2A, 3A, 4A.)

Force ratios (Re) between about 3 and 4 (*e.g.,* a range contained within the area defined by the data points having y-coordinates 2.98, 3.02, 3.29, 3.36, 3.44, 3.73, 4.12) are compatible with speed ratios (SP) between about 4.3 and about 10.7. For an impingement velocity of about 1.72 m/s, this corresponds to an about 400 m/min to about 1000 m/min substrate velocity (U) range. For an adhesive coating composition, this corresponds to a volumetric flow rate (Q) range of about 0.000109 m³/(s*m) to about 0.000711 m³/(s*m). For a release coating composition, this corresponds to a volumetric flow rate (Q) range of about 0.000014 m³/(s*m) to about 0.000067 m³/(s*m). (See Tables 3A, 4A, 5A, 6A and see Graphs 2A, 3A, 4A.)

Force ratios (Re) between about 4 and about 5.20 (*e.g.,* a range contained within the area defined by the data points having y-coordinates 3.73, 4.12, 4.13, 4.47, 4.82, 4.95, 5.22, 5.51) are compatible with speed ratios (SP) between about 5.3 and about 7.5. For an impingement velocity (V) of about 1.72 m/s, this corresponds to an about 500 m/min to about 700 m/min substrate velocity (U) range. For an adhesive coating composition, this corresponds to a volumetric flow rate (Q) range of about 0.000145 m³/(s*m) to about 0.000924 m³/(s*m). For a release coating composition, this corresponds to a volumetric flow rate (Q) range of about 0.000018 m³/(s*m) to about 0.000087 m³/(s*m). (See Tables 3A, 4A, 5A, 6A and see Graphs 2A, 3A, 4A.)

Additionally, speed ratios (SP) between about 3 and about 4 (*e.g.,* a range contained within the area defined by the data points having y-coordinates 3.21, 4.28) can accommodate force ratios (Re) between about 1.0 and 1.3. Speed ratios (SP) between about 4 and 5 (*e.g.,* a range contained within the area defined by the data points having y-coordinates 3.21, 4.28, 5.35) can accommodate force ratios (Re) between about 1.3 and about 4.1. Speed ratios (SP) between about 5 and about 6 (*e.g.,* a range contained within the area defined by the data points having y-coordinates 4.28, 5.35, 5.81, 6.42) can accommodate low force ratios (Re) between about 1.7 and about 4.5. Speed ratios (SP) between about 6 and about 7 (*e.g.,* a range contained within the area defined by the data points having y-coordinates 5.35,6.42,7.48) can accommodate force ratios (Re) between about 2.0 and about 5.0. Speed ratios (SP) between about 7 and about 8 (*e.g.,* a range contained within the area defined by the data points having y-coordinates 6.42, 7.48, 8.55) can accommodate force ratios (Re) between about 2.3 and 5.2. Speed ratios (SP) between about 8 and about 9 (*e.g.,* a range contained within the area defined by the data points having y-coordinates 7.48, 8.55, 9.62) can accommodate force ratios (Re) between about 2.7 and about 5.2. Speed ratios (SP) between about 9 and about 10 (*e.g.,* a range contained within the area defined by the data points having y-coordinates 8.55,9.62,10.69) can accommodate force ratios (Re) between about 3.0 and about 5.2. (See Tables 3B, 4B, 5B, 6B, and see Graphs 2B, 3B, 4B.)

Because curtain coating was also successful at lower force ratios (Re) for these acute impingement angles, the same curtain-coating equipment, and/or the same equipment set-up, may be used over a wide range of curtain flow characteristics. In other words, the system 10 need not be modified to accommodate runs wherein a curtain 16 will have a relatively low (*i.e.,* less than 5.25) force ratio (Re).

Some component modifications to the system 10 may be necessary to accommodate curtain coating operations with acute impingement angles (θ). For example, when the impingement angle (θ) is equal to 90° (see Figures 1A and 1B), edge guides 40 with a substantially horizontal bottom edge 42 will provide the best fit to the impingement zone 14. (See Figure 6A.) However, when the impingement angle (θ) is less than 90° (see Figures 4A and 4B), edge guides 40 with a slanted bottom edge 42 will provide the best fit to the impingement zone 14. (See Figure 6B.) The slant angle α of the edge guide 40 can approximate the complement of the impingement angle (θ) (*e.g.,* α = 90 - θ.) The vacuum assembly 50 may need to be rotatably mounted relative to an arm 52 to allow the head of the vacuum box 54 to be positioned just upstream of the impingement zone 14 (see Figure 8) and/or the catch pan (not shown) may have to be moved to provide sufficient clearance for the edge guides 40.

Some component modifications to the system 10 may be necessary to accommodate the high flow rates possible with the present invention. For example, the lip 60 of the die 20 may need to be modified to prevent the curtain 16 from having ballistic and/or anti-ballistic trajectories. The lip 60 includes a top surface 62, which is positioned parallel with the slide of the die 20, and a front surface 64, over which the liquid coating flows to form the curtain 16. With low curtain flow rates, the front surface 64 slants inward relative to the top surface 62. (Figure 8A.) With high curtain flow rates, the front surface 64 may need to be shifted outward so that it is positioned substantially perpendicular with the top surface 62. (Figure 8B.)

One may now appreciate that the present invention provides a method for successfully curtain coating a substrate when the impinging curtain has a high force ratio (Re). The present invention makes a high volumetric flow rates (Q) feasible, thereby making a high substrate velocities (U) possible, and thereby best maximizing the productivity of capital-investment curtain coating equipment. Although the invention has been shown and described with respect to certain preferred embodiments, it is evident that equivalent and obvious alterations and modifications will occur to others skilled in the art upon the reading and understanding of this specification. The present invention includes all such alterations and modifications and is limited only by the scope of the following claims.

The present invention provides system for successfully curtain coating a substrate when the impinging curtain has a high force ratio (Re). Thus, with the present invention, high volumetric flow rates (Q) are feasible, thereby making high substrate velocities (U) possible, and thereby best maximizing the productivity of capital-investment curtain coating equipment.

A curtain coating method to form a coating on a substrate of a desired coating weight (ctwt) comprises the steps of conveying the substrate in a downstream direction (D) through an impingement zone, and impinging the substrate with a free-falling curtain in the impingement zone. The force ratio (Re) of the curtain in the impingement zone reflects a relatively high inertia force and/or a relatively low viscous force. Specifically, the force ratio (Re) is greater than about 5.25, greater than about 5.5, greater than about 6.0, greater than about 6.5, greater than about 7.0, greater than about 7.5, and/or greater than about 8.0.

The curtain impinges the substrate at an impingement angle (θ) that is less than 90°. For example, the impingement angle (θ) can be between about 70° and about 50°, between about 65° and about 55°, not greater than about 65°, not greater than about 60°, and/or not greater than about 55°. If the substrate is conveyed around a back-up roller, this impingement orientation can be accomplished by the impingement zone being offset from the top-dead-center of the back-up roller. If the substrate is conveyed between two rollers, this impingement orientation can be accomplished by the rollers being vertically offset.

The substrate is conveyed through the impingement zone at a substrate velocity (U) and the curtain impinges the substrate at an impingement velocity (V). Because the impingement angle (θ) is less than 90°, the substrate velocity (U) has a horizontal component (Uₓ) and a vertical component (U_{y}). Also, the impingement velocity (V) has a component (V⊥) perpendicular to the substrate velocity (U) and a component (V∥) parallel to the substrate velocity (U).

The present invention includes the appreciation that the relevant speed ratio (SP) should be equal to the ratio of the substrate velocity (U) to the perpendicular impingement component (V⊥). This speed ratio (SP) properly represents the velocity shift at the impingement zone as the parallel impingement component (VII) does not necessitate any velocity shift and/or as only the perpendicular impingement component (V⊥) requires a velocity shift.

The present invention also includes the appreciation that vertical component (U_{y}) of the substrate velocity (U) is significant in that it provides downward momentum to the liquid coating composition as it impinges the substrate. This "push" in the impingement zone is believed to prevent the heel formation and/or air entrapment which would otherwise occur at high force ratios. I n a curtain coating method according to the present invention, the speed ratio (SP) is greater than about 7.0 and less than about 12.0. More specifically, when the force ratio (Re) is less than about 6, the speed ratio (SP) is between about 7.5 and about 9.5 (corresponding to a substrate speed (U) in a range of about 700 m/min to about 800 m/min when the impingement velocity (V) is about 1.72 m/s). When the force ratio (Re) is between about 6 and 7, the speed ratio (SP) is between about 8.6 and about 11.9 (corresponding to a substrate velocity (U) range of about 800 m/min to about 1000 m/min when the impingement velocity (V) is about 1.72 m/s). When the force ratio (Re) is between 7 and 8 and the speed ratio (SP) is between about 9.6 and about 11.9 (corresponding to a substrate velocity (U) range of about 900 m/min to about 1000 m/min when the impingement velocity is about 1.72 m/s). When the force ratio (Re) is greater than 8, the speed ratio (SP) is greater than 10 (corresponding to a substrate speed (U) of at least about 1000 m/min when the impingement speed (V) is about 1.72 m/s).

For an adhesive coating composition (*e.g*. a coating composition having a density (p) between about 900 kg/m³ and about 1100 kg/m³ and having a viscosity (η) between about 0.040 Pa s and about 0.160 Pa s) volumetric flow rates (Q) in excess of 0.000900 m³/s*m are possible. Specifically, for example, volumetric flow rates (Q) of about 0.000189 m³/(s*m) to about 0.00107 m³/(s*m) are possible (when the force ratio (Re) is from about 5.2 to about 6.0 and/or the speed ratio (SP) is between about 7.5 and about 9.5); volumetric flow rates (Q) of about 0.000218 m³/(s*m) to about 0.00124 m³/(s*m) are possible (when the force ratio (Re) is between about 6.0 and about 7.0 and/or the speed ratio (SP) is between about 8.6 and about 11.9); volumetric flow rates (Q) of about 0.000255 m³/(s*m) to about 0.00142 m³/(s*m) are possible (when the force ratio (Re) is between about 7.0 and about 8.0 and/or the speed ratio (SP) is between about 9.6 and 11.9); and volumetric flow rates (Q) as high as 0.0147 m³/(s*m) are possible (when the force ratio (Re) is above about 8.0 and/or the speed ratio (SP) is between about 10.7 and 11.9).

For a release or other low viscosity composition (*e.g*. a coating composition having a density (p) between about 900 kg/m³ and about 1100 kg/m³ and having a viscosity (η) between about 0.005 Pa s and about 0.015 Pa s) volumetric flow rates (Q) in excess of 0.000090 m³/s*m are possible. Specifically, for example, volumetric flow rates (Q) from about 0.000024 m³/(s*m) to about 0.000100 m³/(s*m) are possible (when the force ratio (Re) is from about 5.2 to about 6.0 and/or when the speed ratio (SP) is between about 7.5 and about 9.5); volumetric flow rates (Q) from about 0.000027 m³/(s*m) to about 0.000117 m³/(s*m) are possible (when the force ratio (Re) is between about 6 and about 7 and/or when the speed ratio (SP) is between about 8.6 and about 11.9); volumetric flow rates (Q) of about 0.000032 m³/(s*m) to about 0.000133 m³/(s*m) are possible (when the force ratio (Re) is between about 7 and about 8 and/or the speed ratio (SP) is between about 9.6 and about 11.9); and volumetric flow rates (Q) above 0.000136 m³/(s*m) are possible (when the force ratio (Re) is above 8 and/or the speed ratio (SP) is between about 10.7 and about 11.9).

## Claims

1. A curtain coating system (10) for applying a coating on a substrate (12), comprising a conveyor (22/24) that conveys the substrate (12) in a downstream direction (D) through an impingement zone (14), and a free-falling curtain (16) that impinges the substrate (12) in the impingement zone (14) at an impingement angle (θ) to form a coating (18) on the substrate (12) of a desired coating weight (ctwt); wherein:
said system is suitable for providing an impingement angle (θ) of less than 90°;
**characterized in that**
said system is suitable for providing a force ratio (Re) of greater than about 5.25, said force ratio being defined as the ratio of the mass flow rate per unit width of the curtain (16) to the viscosity of the liquid coating composition ;
such that the coating (18) has a thickness (t_{w}) that varies less than 2% from a predetermined uniform final coating thickness (too) over the width (w) of the coating (18).
wherein said system further comprises a die lip (60) including a top surface (62), which is positioned parallel to a slide surface of a die (20) and a front surface (64) over which the liquid coating composition flows to form the curtain (16), and wherein the front surface (64) is positioned substantially perpendicular to the top surface (62).

2. A curtain coating system (10) according to claim 1, wherein the conveyor comprises a back-up roller (22) and wherein the impingement zone (14) is offset in the downstream direction (D) from a top-dead-center of the back-up roller (22).

3. A curtain coating system (10) according to claim 1 or 2, wherein the conveyor comprises a pair of conveying rollers (24) vertically offset in the downstream direction (D) and wherein the impingement zone (14) is positioned between the rollers (24).

4. A curtain coating system (10) according to any one or more of the preceding claims, further comprising edges guides (40) with bottom surfaces (42), the bottom surfaces (42) being slanted in a downward direction at a slant angle (α) approximately equal to the complement of the impingement angle (θ).

5. A curtain coating system (10) according to any one or more of the preceding claims, further comprising a vacuum assembly (50) having a rotatably mounted vacuum box (54).

6. A curtain coating system (10) according to any one or more of the preceding claims, wherein said system is suitable for providing said impingement angle (θ) between 70° and 50°, at the best between 65° and 55°.

7. A curtain coating system (10) according to any one or more of the preceding claims, wherein said system is suitable for providing a force ratio (Re) of greater than 6.00, preferably greater than 7.00, at the best greater than 8.00.

8. A curtain coating system (10) according to any one or more of the preceding claims, wherein said system is suitable for providing a velocity (U) of said substrate that is between 700 m/min and 1000 m/min, preferably greater than about 800 m/min, at the best greater than about 900 m/min.

9. A curtain coating system (10) according to claim 8, wherein said system is suitable for providing a horizontal component (Ux) of the velocity (U) between about 570 m/min and 910 m/min.

10. A curtain coating system (10) according to any one or more of the preceding claims 8 or 9, wherein said system is suitable for providing a vertical component (Uy) of the substrate velocity between about 300 m/min and about 600 m/min.

11. A curtain coating system (10) according to any one or more of the preceding claims 8 to 10, wherein said system is suitable for providing a speed ratio (SP) greater than about 7.0 and less than 12.00.

## Patentansprüche

1. Vorhangbeschichtungssystem (10) zum Aufbringen einer Beschichtung auf einem Substrat (12), das umfasst: einen Förderer (22/24), der das Substrat (12) in eine laufabwärtige Richtung (D) durch eine Aufprallzone (14) befördert, und einen freifallenden Vorhang (16), der in der Aufprallzone (14) in einem Aufprallwinkel (θ) auf das Substrat (12) aufprallt, um eine Beschichtung (18) mit einem gewünschten Beschichtungsgewicht (ctwt) auf dem Substrat (12) zu bilden;
wobei:
das System geeignet ist, einen Aufprallwinkel (θ) von weniger als 90° bereitzustellen;
**dadurch gekennzeichnet, dass**
das System geeignet ist, um ein Kraftverhältnis (Re) von mehr als etwa 5,25 bereitzustellen, wobei das Kraftverhältnis als das Verhältnis des Massendurchsatzes pro Einheitsbreite des Vorhangs (16) zu der Viskosität der flüssigen Beschichtungszusammensetzung definiert ist;
so dass die Beschichtung (18) eine Dicke (t_{w}) hat, die über die Breite (w) der Beschichtung (18) weniger als 2% von einer vorgegebenen einheitlichen abschließenden Beschichtungsdicke (t_{∞}) abweicht,
wobei das System ferner eine Austrittslippe (60) umfasst, die umfasst: eine obere Fläche (62), die parallel zu einer Gleitfläche eines Ausformwerkzeugs (20) positioniert ist, und eine vordere Fläche (64), über welche die flüssige Beschichtungszusammensetzung fließt, um den Vorhang (16) zu bilden, und wobei die vordere Fläche (64) im Wesentlichen senkrecht zu der oberen Oberfläche (62) positioniert ist.

2. Vorhangbeschichtungssystem (10) nach Anspruch 1, wobei der Förderer einen Stützpresseur (22) umfasst, und wobei die Aufprallzone (14) in der Laufabwärtsrichtung (D) gegen einen oberen Totpunkt des Stützpresseurs (22) versetzt ist.

3. Vorhangbeschichtungssystem (10) nach Anspruch 1 oder 2, wobei der Förderer ein Paar von Förderwalzen (24) umfasst, die in der Laufabwärtsrichtung (D) vertikal versetzt sind, und wobei die Aufprallzone (14) zwischen den Walzen (24) positioniert ist.

4. Vorhangbeschichtungssystem (10) nach einem oder mehreren der vorhergehenden Ansprüche, das ferner Kantenführungen (40) mit unteren Flächen (42) umfasst, wobei die unteren Flächen (42) in einer Abwärtsrichtung in einem Schrägwinkel (α) geneigt sind, der ungefähr gleich dem Komplement des Aufprallwinkels (θ) ist.

5. Vorhangbeschichtungssystem (10) nach einem oder mehreren der vorhergehenden Ansprüche, das ferner eine Vakuumanordnung (50) umfasst, die eine drehbar montierte Vakuumkammer (54) hat.

6. Vorhangbeschichtungssystem (10) nach einem oder mehreren der vorhergehenden Ansprüche, wobei das System geeignet ist, um den Aufprallwinkel (θ) zwischen 70° und 50°, am besten zwischen 65° und 55°, bereitzustellen.

7. Vorhangbeschichtungssystem (10) nach einem oder mehreren der vorhergehenden Ansprüche, wobei das System geeignet ist, um ein Kraftverhältnis (Re) von mehr als 6,00, bevorzugt mehr als 7,00, am besten mehr als 8,00, bereitzustellen.

8. Vorhangbeschichtungssystem (10) nach einem oder mehreren der vorhergehenden Ansprüche, wobei das System geeignet ist, eine Geschwindigkeit (U) des Substrats bereitzustellen, die zwischen 700 m/Min und 1000 m/Min, vorzugsweise bei mehr als etwa 800 m/Min, am besten bei mehr als etwa 900 m/Min, liegt.

9. Vorhangbeschichtungssystem (10) nach Anspruch 8, wobei das System geeignet ist, eine horizontale Komponente (Ux) der Geschwindigkeit (U) zwischen etwa 570 m/Min und 910 m/Min bereitzustellen.

10. Vorhangbeschichtungssystem (10) nach einem oder mehreren der vorhergehenden Ansprüche 8 oder 9, wobei das System geeignet ist, eine vertikale Komponente (Uy) der Substratgeschwindigkeit (U) zwischen etwa 300 m/Min und 600 m/Min bereitzustellen.

11. Vorhangbeschichtungssystem (10) nach einem oder mehreren der vorhergehenden Ansprüche 8 bis 10, wobei das System geeignet ist, ein Geschwindigkeitsverhältnis (SP) von mehr als etwa 7,0 und weniger als 12,00 bereitzustellen.

## Revendications

1. Système d'enduction au rideau (10) pour appliquer un revêtement sur un substrat (12), comprenant un convoyeur (22/24) qui transporte le substrat (12) dans une direction en aval (D) à travers une zone de choc (14) et un rideau en chute libre (16) qui se heurte contre le substrat (12) dans la zone de choc (14) à un angle de choc (θ) pour former un revêtement (18) sur le substrat (12) d'un poids de revêtement souhaité (ctwt) ;
dans lequel :
ledit système convient à fournir un angle de choc (θ) inférieur à 90° ;
**caractérisé en ce que**
ledit système convient à fournir un rapport de force (Re) supérieur à environ 5,25, ledit rapport de force étant défini comme le rapport du débit massique par largeur unitaire du rideau (16) à la viscosité de la composition de revêtement liquide ;
de sorte que le revêtement (18) a une épaisseur (t_{w}) qui varie de moins de 2 % d'une épaisseur de revêtement final uniforme prédéterminée (t∞) sur la largeur (w) du revêtement (18) ;
dans lequel ledit système comprend en outre une lèvre de filière (60) incluant une surface supérieure (62) qui est positionnée parallèlement à une surface de coulissement d'une filière (20) et une surface avant (64) sur laquelle la composition de revêtement liquide s'écoule pour former le rideau (16), et dans lequel la surface avant (64) est positionnée essentiellement perpendiculairement à la surface supérieure (62).

2. Système d'enduction au rideau (10) selon la revendication 1, dans lequel le convoyeur comprend un cylindre d'appui (22) et dans lequel la zone de choc (14) est décalée dans la direction en aval (D) depuis un point mort haut du cylindre d'appui (22).

3. Système d'enduction au rideau (10) selon la revendication 1 ou 2, dans lequel le convoyeur comprend une paire de cylindres d'appui (24) décalés verticalement dans la direction en aval (D) et dans lequel la zone de choc (14) est positionnée entre les cylindres (24).

4. Système d'enduction au rideau (10) selon l'une quelconque ou plusieurs des revendications précédentes, comprenant en outre des guides de bord (40) avec des surfaces inférieures (42), les surfaces inférieures (42) étant inclinées dans une direction vers le bas à un angle d'inclinaison (α) approximativement égal au complément de l'angle de choc (θ).

5. Système d'enduction au rideau (10) selon l'une quelconque ou plusieurs des revendications précédentes, comprenant en outre un ensemble d'aspiration (50) ayant une caisse aspirante montée à rotation (54).

6. Système d'enduction au rideau (10) selon l'une quelconque ou plusieurs des revendications précédentes, dans lequel ledit système convient à fournir ledit angle de choc (θ) entre 70° et 50°, au mieux entre 65° et 55°.

7. Système d'enduction au rideau (10) selon l'une quelconque ou plusieurs des revendications précédentes, dans lequel ledit système convient à fournir un rapport de force (Re) supérieur à 6,00, de préférence supérieur à 7,00, au mieux supérieur à 8,00.

8. Système d'enduction au rideau (10) selon l'une quelconque ou plusieurs des revendications précédentes, dans lequel ledit système convient à fournir une vitesse (U) dudit substrat qui est comprise entre 700 m/min et 1000 m/min, de préférence supérieure à environ 800 m/min, au mieux supérieure à environ 900 m/min.

9. Système d'enduction au rideau (10) selon la revendication 8, dans lequel ledit système convient à fournir une composante horizontale (Ux) de la vitesse (U) comprise entre environ 570 m/min et 910 m/min.

10. Système d'enduction au rideau (10) selon l'une quelconque ou plusieurs des revendications précédentes 8 ou 9, dans lequel ledit système convient à fournir une composante verticale (Uy) de la vitesse du substrat comprise entre environ 300 m/min et environ 600 m/min.

11. Système d'enduction au rideau (10) selon l'une quelconque ou plusieurs des revendications précédentes 8 à 10, dans lequel ledit système convient à fournir un rapport de vitesse (SP) supérieur à environ 7,0 et inférieur à 12,00.
